

[54] COLOR PHOTOGRAPHIC DEVELOPING  
METHOD AND DEVELOPER THEREFOR[75] Inventors: **Fumio Hasegawa; Takeo Emoto; Satoshi Kurihara**, all of Kanagawa, Japan[73] Assignee: **Fuji Photo Film Co., Ltd.,** Kanagawa, Japan[22] Filed: **Aug. 18, 1972**[21] Appl. No.: **281,673**

## [30] Foreign Application Priority Data

Aug. 20, 1971 Japan ..... 46/63432

[52] U.S. Cl. .... **96/66 R**, 96/66.4, 96/22,  
96/55 XR[51] Int. Cl. .... **G03c 5/30**, G03c 7/16[58] Field of Search ..... 96/66.4, 22, 166,  
96/66

## [56] References Cited

## UNITED STATES PATENTS

2,091,689 8/1937 Russell ..... 96/66.4

|           |         |                   |         |
|-----------|---------|-------------------|---------|
| 2,138,486 | 11/1938 | Fournes .....     | 96/66.4 |
| 2,193,015 | 3/1940  | Weissberger ..... | 96/66 R |
| 2,366,496 | 1/1945  | Dawson .....      | 96/66.4 |
| 3,615,497 | 10/1971 | Fassbender .....  | 96/66.1 |

## OTHER PUBLICATIONS

Chem. Absts. Vol. 51, 13627e-f-g.

Primary Examiner—Norman G. Torchin

Assistant Examiner—M. F. Kelley

Attorney—Richard C. Sughrue et al.

## [57] ABSTRACT

In a color photographic developing method of silver halide color photographic materials by developing said materials with a developer solution containing 4-amino-3-methyl-N-ethyl-N-( $\beta$ -methanesulfonamidoethyl)aniline sesquisulfate monohydrate as a developing agent, the crystallization of the developing agent in the developer solution is prevented by incorporating at least one crystallization preventing agent selected from the group consisting of lactose and hydroxypropylmethyl cellulose into the developer solution.

6 Claims, No Drawings

## COLOR PHOTOGRAPHIC DEVELOPING METHOD AND DEVELOPER THEREFOR

### BACKGROUND OF THE INVENTION

#### 1. FIELD OF THE INVENTION

This invention relates to a color photographic developing method and a developer therefor and, more particularly, it relates to a method for developing a silver halide color photographic material with a developer containing 4-amino-3-methyl-N-ethyl-N-( $\beta$ -methanesulfonamidoethyl)aniline sesquisulfate monohydrate (hereinafter referred to as a developing agent) and a crystallization preventing agent for an amine base of the developing agent.

#### 2. DESCRIPTION OF THE PRIOR ART

As described in prior arts, it is known that an amine base of the developing agent cannot advantageously be used because it is crystallized out at a low temperature. This disadvantage is due to the salt out of the developing agent by an inorganic substance such as sodium carbonate or sodium sulfate incorporated in the developer solution.

An object of the present invention is therefore to provide a color developing method without accompanying with the crystallization of the developing agent.

Another object of the present invention is to provide a color photographic developer of which the crystallization is prevented.

### SUMMARY OF THE INVENTION

As a result of research for eliminating the above-described disadvantage, it was found that the above objects can be attained by incorporating at least a member selected from the group consisting of lactose and hydroxypropylmethyl cellulose as a crystallization-preventing agent into a color photographic developer solution containing the developing agent.

Generally, crystallization-preventing agents must have an appropriate solubility in photographic developer solution and must not adversely effect the photographic properties of the color photographic materials to be developed. In these points, lactose and hydroxypropylmethyl cellulose are preferable crystallization-preventing agents because they satisfy the above requirements. For example, hydroxylpropylmethyl cellulose used in the present invention has less tendency to be salted out in the developer solution than methyl cellulose described in the specification of Japapese Patent Publication No. 41,476/71. That is, while the addition of methyl cellulose in an amount of more than 0.7 percent by weight based on the developing agent to the developer solution increases the crystallization-preventing effect, methyl cellulose per se is salted out to produce the precipitate thereof. On the other hand, hydroxypropylmethyl cellulose is not salted out even if it is added in an amount of 1 percent by weight based on the developing agent. The crystallization-preventing agent of the invention can be incorporated in the powder form into the developing agent in the form of powder, particle or granule, or can be incorporated as a powder form or an aqueous solution into the developer solution at any stage, for example, in preparing the developer solution or after the developer solution has been prepared for use.

The amount of the crystallization-preventing agent can range from 0.1 to 1.0 percent by weight, preferably

from 0.4 to 1.0 percent by weight based on the developing agent.

A photographic developer solution of the present invention may contain conventional photographic additives such as preservatives, development-promoting agents, development inhibitors, antifoggants or alkalis.

### EXAMPLE 1

A sensitometric exposure using a sensitometer was 10 applied to a multiple-layer color negative film containing an anti-diffusion color coupler.

Then, three pieces of the color negative film thus exposed were subjected to a developing treatment using 15 three kinds of developer solution, i.e., Developer A without any crystallization-preventing agent added and which was prepared for the purposes of comparison, Developer B containing lactose, and Developer C containing hydroxypropylmethyl cellulose.

|   | Treating Process  | Temperature | Time    |
|---|-------------------|-------------|---------|
| 1 | Color Development | 20°C        | 10 min. |
| 2 | First Fixation    | 20°C        | 5 min.  |
| 3 | Rinsing           | 16°-20°C    | 5 min.  |
| 4 | Bleaching         | 20°C        | 5 min.  |
| 5 | Rinsing           | 16°-20°C    | 5 min.  |
| 6 | Second Fixation   | 20°C        | 5 min.  |
| 7 | Rinsing           | 16°-20°C    | 8 min.  |
| 8 | Drying            | Below 35°C  | —       |

The compositions of the Developers A, B, and C employed in the above treatment were as follows;

|                                | DEVELOPER A       |
|--------------------------------|-------------------|
| Anhydrous Sodium Sulfite       | 2.0 g             |
| Developing Agent               | 5.0 g             |
| Sodium Carbonate (monohydrate) | 50 g              |
| Potassium Bromide              | 2.0 g             |
| Sodium Hydroxide               | 1.0 g             |
| Water was added to make        | 1.0 l of solution |

### DEVELOPER B

The same composition as Developer A was employed 40 except 1.0 percent by weight of lactose based on the developing agent was additionally added.

### DEVELOPER C

The same composition as Developer A was employed 45 except 1.0 percent by weight of hydroxypropylmethyl cellulose based on the developing agent was additionally added.

The results of the development employing Developers A, B, and C were such that there were no differences between each of the developers with respect to 50 the red, green, and blue relative sensitivity, gamma ( $\bar{G}$ ), and fog, respectively, as a result of the differences between the Developers A, B, and C, and the resulting photographic properties were normal, respectively.

### EXAMPLE 2

A developer solution was prepared employing the same kind of developing agent used in Example 1 in accordance with the following formulation. In the course of the preparation of the developer solution, lactose and/or hydroxypropylmethyl cellulose was added in several different quantities, respectively. Each of the resulting developer solutions was settled at a temperature of from 15° to 16°C.

#### Developer Composition

|                                  |
|----------------------------------|
| Water (25° - 30°C) — 800ml       |
| Anhydrous Sodium Sulfite — 2.0 g |
| Crystallization Preventing Agent |

Lactose<sup>(1)</sup>—0.037 g—0.065 g

or

Hydroxypropylmethyl Cellulose<sup>(2)</sup> — 0.0065 g — 0.065 g

Developing Agent<sup>(3)</sup> — 6.5 g

Sodium Carbonate (Monohydrate) — 60 g

Potassium Bromide — 2.0 g

Sodium Hydroxide — 1.0 g

Water was added to make 1.0 l of solution

(1) Commercially available lactose according to the pharmacopoeia of Japan at a level of 0.5 percent and 1 percent by weight with respect to the amount of the developing agent was employed.

(2) 1 g of hydroxypropylmethyl cellulose was dissolved in 50 ml of water to obtain solution, 0.1, 0.05, and 1.0 percent each of the resulting solution based on the developing agent was added thereto.

the viscosity of a 2 percent aqueous solution of hydroxypropylmethyl cellulose at a temperature of 20°C was 7.2 — 4.8 CPS.

(3) The developing agent was prepared through decoloration with activated charcoal and recrystallization in a dilute sulfuric acid methanol from which the developing agent could be easily salted out.

The results of the effects for preventing the crystallization of the developing agent are shown in the following table from which it can be understood that the solubility of the developing agent was elevated by adding the lactose and/or the hydroxypropylmethyl cellulose, whereby crystallization of the developing agent was effectively prevented.

TABLE

| Crystallization Preventing Agent   | Time required for Separating Crystals of Amine Base (16°C) (hr.) | Note                                                                           |
|------------------------------------|------------------------------------------------------------------|--------------------------------------------------------------------------------|
| Without Addition                   | $t \leq 1$                                                       | A large amount of developing agent crystallized out                            |
| Lactose 0.5%                       | $t > 48$                                                         |                                                                                |
| Lactose 1.0%                       | $t > 48$                                                         |                                                                                |
| Hydroxypropylmethyl Cellulose 0.1% | $24 < t < 48$                                                    | After 48 hours, an extremely small amount of developing agent crystallized out |
| Hydroxypropylmethyl Cellulose 0.5% | $t > 48$                                                         |                                                                                |
| Do. 1.0%                           | $t > 48$                                                         |                                                                                |

While the invention has been described in detail and with reference to specific embodiments thereof, it will be apparent that various changes and modifications can be made therein without departing from the spirit scope thereof.

What is claimed is:

1. In a color photographic developing method of silver halide color photographic materials by developing said materials with a developer solution containing 4-amino-3-methyl-N-ethyl-N-( $\beta$ -methanesulfonamidoethyl)aniline sesquisulfate monohydrate as a developing agent, the improvement which comprises preventing the crystallization of the developing agent in the developer solution by incorporating at least one crystallization-preventing agent selected from the group consisting of lactose and hydroxypropylmethyl cellulose into the developer solution.

2. The method as claimed in claim 1, wherein the amount of said crystallization-preventing agent is in the range of from 0.1 to 1.0 percent by weight based on the weight of said developing agent.

3. The method as claimed in claim 2, wherein said amount is from 0.4 to 1.0 percent by weight based on the weight of said developing agent.

4. A color developer solution comprising 4-amino-3-methyl-N-ethyl-N-( $\beta$ -methanesulfonamidoethyl)aniline sesquisulfate monohydrate as a developing agent and at least one crystallization-preventing agent selected from the group consisting of lactose and hydroxypropylmethyl cellulose.

5. The color developer solution as claimed in claim 4, wherein the amount of said crystallization-preventing agent is in the range of from 0.1 to 1.0 percent by weight based on the weight of said developing agent.

6. The color developer solution as claimed in claim 5, wherein said amount is from 0.4 to 1.0 percent by weight based on the weight of said developing agent.

\* \* \* \* \*